

# United States Patent [19]

Birke

[11] 3,880,879

[45] Apr. 29, 1975

[54] DIBENZIMIDAZOLE COMPOUNDS

[75] Inventor: August H. Birke, Godfrey, Ill.

[73] Assignee: Shell Oil Company, New York, N.Y.

[22] Filed: Sept. 27, 1973

[21] Appl. No.: 401,516

Related U.S. Application Data

[60] Division of Ser. No. 296,733, Oct. 11, 1972, Pat. No. 3,785,979, which is a continuation-in-part of Ser. No. 169,459, Aug. 5, 1971, abandoned.

[52] U.S. Cl. .... 260/309.2

[51] Int. Cl. .... C10m 5/20

[58] Field of Search ..... 260/309.2

[56] References Cited

UNITED STATES PATENTS

|           |         |                |            |
|-----------|---------|----------------|------------|
| 3,105,837 | 10/1963 | Ursprung ..... | 260/309.2  |
| 3,752,765 | 8/1973  | Birke .....    | 252/51.5 A |
| 3,785,979 | 1/1974  | Birke .....    | 252/51.5 A |

Primary Examiner—Henry R. Jiles

Assistant Examiner—C. M. S. Jaissle

Attorney, Agent, or Firm—Henry C. Geller

[57] ABSTRACT

Dibenzimidazole compounds corresponding to the formula:



wherein R<sub>1</sub> and R<sub>2</sub> are aliphatic hydrocarbyl radicals, R<sub>3</sub> is a hydrocarbylene radical, R<sub>4</sub> and R<sub>5</sub> are aromatic hydrocarbyl radicals and X is —O— or



are highly efficacious grease thickening agents.

8 Claims, No Drawings

## DIBENZIMIDAZOLE COMPOUNDS

## CROSS-REFERENCE TO RELATED APPLICATIONS

This is a division of application Ser. No. 296,733, filed Oct. 11, 1972, now U.S. Pat. No. 3,785,979, patented Jan. 15, 1974, which application is a continuation-in-part of copending U.S. application Ser. No. 169,459, filed Aug. 5, 1971, now abandoned.

## BACKGROUND OF THE INVENTION

## 1. Field of the Invention

This invention relates to a novel class of dibenzimidazole compounds and grease compositions gelled therewith.



## 2. Description of the Prior Art

It has become increasingly important that grease composition be able to provide adequate lubrication at high temperatures, e.g., temperatures of 350°F to 450°F or higher. Numerous thickening agents have been proposed for use in such greases, including soap base thickeners, inorganic clay thickeners and organic thickening agents. Examples of this latter class of thickening agents include various polyureas, ureido compounds, aminoaryl diureas, triazines and the like. Such organic thickening agents are typically prepared by reacting one or more mono-, di-, or polyamines with one or more mono-, di-, or polyisocyanates. Other related organic thickeners include arylcarbamyl compounds formed by reacting an aromatic amine with the reaction product of an aromatic diisocyanate and p-aminobenzoic acid.

While organic thickening agents of the aforementioned types produce greases having desirably high dropping points, this is but one measure of a grease's ability to perform satisfactorily at high temperatures. Other important properties include thermal and mechanical stability, high temperature bearing performance, oxidation and corrosion resistance, etc. While additives are normally incorporated into grease compositions to improve one or more of these properties, the thickening agent itself can significantly affect, either favorably or adversely, the properties of the finished

grease product. Thus, in spite of the numerous organic thickening agents known in the art, there is a continuing need for the development of thickening agents which will not only produce greases having high dropping points, but which will additionally augment other important properties of the finished product. The present invention provides such a class of thickening agents.

## 10 SUMMARY OF THE INVENTION

It has now been found that grease compositions having excellent high temperature lubricating properties can be produced by incorporating into an oleaginous base vehicle, a minor amount of a dibenzimidazole compound corresponding to the formula:



wherein R<sub>1</sub> and R<sub>2</sub> are aliphatic hydrocarbyl radicals, R<sub>3</sub> is a hydrocarbylene radical, R<sub>4</sub> and R<sub>5</sub> are aromatic hydrocarbylene radicals and X is —O— or

25 30 Not only do the grease compositions of the invention have high dropping points, but in addition they have excellent mechanical and thermal stability, and high temperature bearing performance properties as well. These excellent qualities are believed attributable in large part to the unique dibenzimidazole structure of the present thickening agents which produces as extremely stable molecule.

## 40 DESCRIPTION OF THE PREFERRED EMBODIMENTS

The aforescribed dibenzimidazole thickening agents can be conveniently prepared by reacting one mole of a dicarboxylic acid anhydride with two moles of a nitro-substituted phenylenediamine, followed by reduction of the nitro groups to amine groups, and further reaction with two moles of the reaction product of an aromatic diisocyanate with a monohydric alcohol or monoamine. This procedure is illustrated by the following equations:

Equation 1



Equation 2



Equation 3



Equation 4

Preparation of Dibenzimidazole-Urea Thickeners

Equation 5



Equation 6



An alternative method of preparing the bis-nitrobenzimidazole (intermediate product I) employed in Equation 2, is to react the dicarboxylic acid or its anhydride with two moles of a phenylene diamine which is not nitro-substituted. The resultant product can be subsequently nitrated to produce bis-nitrobenzimidazole which is then converted to its amino form (intermediate product II) and reacted with two moles of intermediate products III or V as shown in Equations 4 and 6, respectively. A more detailed description of the preparation of the benzimidazole thickeners is given in the examples.

Dicarboxylic acids or anhydrides which can be suit-

ably employed in preparing the thickeners of the invention include the acids or anhydrides of aliphatic dicarboxylic acids such as succinic, glutaric, adipic, pimelic, suberic, azelaic, sebatic acids or anhydrides, as well as the anhydrides of aromatic dicarboxylic acids such as phthalic, isophthalic or terephthalic acids or anhydrides or their esters. Cyclohexane dicarboxylic acids and anhydrides such as 1,2- or 1,4-cyclohexane dicarboxylic acid or anhydride are likewise suitable as is tetrahydrophthalic acid or anhydride. Hydrocarbyl substituted dicarboxylic acid anhydrides can also be employed, for example, alkyl- or alkenyl-substituted succinic corresponding to the formula



is an alkyl or alkenyl substituent of from one to 16 carbon atoms or more. Aliphatic dicarboxylic acid anhydrides are preferred, and in general are selected so that the  $R_3$  radical of the previously depicted formula has from 2 to 20, preferably from 2 to 12 carbon atoms.

Phenylene diamines suitable for preparing the thickening agents of the invention are ortho-phenylene diamines having a nitro group substituted thereon, e.g., 4-nitro-o-phenylene diamine. In addition to the nitro substituent, o-phenylene diamines having other substituents, e.g., alkyl or halo substituents, can also be employed provided that such substituents do not appreciably interfere with the reaction of the phenylene diamine with the dicarboxylic acid anhydride.

If the alternative procedure discussed above is employed to prepare the bis-nitrobenzimidazole intermediate, the phenylene diamine need not contain a nitro substituent since the addition of the nitro groups is accomplished subsequent to formation of the bis-benzimidazole. Hence, when this procedure is followed, unsubstituted o-phenylene diamine may be utilized or any other o-phenylene diamine having substituents which will not appreciably interfere with the formation of bis-benzimidazole or its subsequent nitration. Specific examples of such phenylene diamines include 4-chloro-o-phenylene diamine and 3,4-toluene diamine.

Aromatic diisocyanates which may be employed in accordance with the invention include mono or di-nuclear aromatic diisocyanates having a total of from 40 six to 20 carbon atoms. Such diisocyanates include biphenylenediisocyanates, naphthylenediisocyanates and monophenylenediisocyanates including tolylenediisocyanate. Illustrative of such diisocyanates are 3,3-dimethylbiphenyl-4,4'-diisocyanate diphenylmethane-4,4'-diisocyanate, 3,3-dimethyldiphenylmethane-4,4'-diisocyanate, 2,4-tolylenediisocyanate, 1,5-naphthylenediisocyanate and mixtures of 2,4- and 2,6-tolylenediisocyanates. 2,4-Tolylenediisocyanate and mixtures of 2,4- and 2,6-tolylenediisocyanates are particularly preferred diisocyanate reactants.

Monohydric alcohols which can be suitably employed to prepare the dibenzimidazole-diurethane-diurea thickeners include aliphatic alcohols having from eight to 30, preferably from 12 to 24, carbon atoms. Examples of such alcohols include octyl, nonyl, lauryl, tetradecyl, hexadecyl, octadecyl, octadecenyl, eicosyl and docosyl alcohols, etc., and mixtures thereof. Thickeners prepared using stearyl or oleyl alcohols or mixtures thereof have been found to be particularly advantageous.

Monoamines which can be employed to prepare the dibenzimidazole-urea thickeners of the invention are aliphatic monoamines or those having a predominantly aliphatic character having from eight to 30, preferably from 12 to 24, carbon atoms. Suitable monoamines include octylamine, decylamine, dodecylamine, tet-

radecylamine, hexadecylamine, heptadecylamine, octadecylamine, octadecenylamine, eicosylamine, docosylamine, tetracosylamine, etc. and mixtures thereof.

5 Mixtures of the above-mentioned monohydric alcohols and monoamines can also be employed thereby producing benzimidazole compounds having both alkylurethane and alkylurylene terminal groups.

The thickening agents of the invention are generally employed in grease compositions in an amount sufficient to gel the oleaginous base vehicle to grease consistency. This amount can vary, for example, from about 5-50% by weight of the total composition. Normally, however, thickener concentrations of 10-35% by weight are sufficient to impart the desired consistency to the inventive compositions.

A wide variety of lubricating oils may be employed as the base vehicle in the present compositions. Suitable base oils include mineral lubricating oils such as naphthenic base, paraffin base or mixed base oils having a viscosity in the range of from 50 SSU at 100°F to 300 SSU at 210°F; synthetic hydrocarbon oils such as oligomerized alpha-olefins and oils derived from coal products; synthetic oils such as alkylene polymers, alkylene oxide-type polymers, polyalkene glycols, polyethers, phosphate esters, dicarboxylic acid esters and pentaerythritol esters. The above oils may be used individually or in mixtures thereof, wherever miscible or made so by the use of solvents. Of the aforementioned base oils, mineral lubricating oils having viscosities of from about 400 to 700 SSU at 100°F are especially preferred.

In addition to the dibenzimidazole thickeners, the present compositions can also contain anti-corrosion additives such as disodium sebacate, glyceryl monooleate, sodium sulfonates, sodium nitrite, amino- and benzo-triazoles, and isostearamides or imidazolines of tetraethylenepentamine; oxidation inhibitors such as phenyl-alpha-naphthylamine, phenyl-beta-naphthylamine, diphenylamines, phenothiazine, dithiocarbamates and various analogs and homologs thereof; viscosity index improvers such as methacrylate polymers and copolymers; extreme pressure agents, and any other additive recognized in the art to perform a particular function or functions.

The following examples illustrate the method of preparation of the present thickeners and their excellent properties. It is to be understood, however, that these examples are presented for illustrative purposes only and that the invention in its broader aspects should not be limited thereto.

#### EXAMPLE I

##### Preparation of Dibenzimidazole-Urea-Urethane Thickening Agents

A 4-liter round bottom flask was charged with 302.2 g (2 moles) of 4-nitro-o-phenylene diamine, 100.0 g (1 mole) of succinic anhydride and 2 liters of 4 normal hydrochloric acid solution. The flask and its contents were then refluxed, with stirring for 24 hours. Heating was discontinued when the reactants were cooled to 0°C, filtered, and the filtrate was discarded. The precipitate was collected and neutralized with 1,500 ml of 5 normal ammonium hydroxide solution, refiltered, and washed twice with water. The neutralized material resulting was dissolved in refluxing ethylene glycol, treated with decolorizing charcoal, filtered and the fil-

trate cooled. The crystalline precipitate that appeared was collected, washed with ethanol and dried. The yield was 65 grams of 1,2-bis(5-nitrobenzimidazoyl-2)ethane having a melting point of 305°C.

56.04 g (0.16 mole) of the above product was then suspended in 1,200 ml of 3 normal hydrochloric acid solution to which was added palladium on charcoal catalyst and reduction of the nitro groups effected in a low pressure hydrogenation apparatus. The catalyst was then filtered off, the filtrate neutralized with sodium bicarbonate and the resulting precipitate collected. After washing with water and drying, 41.5 g of 1,2-bis(5-aminobenzimidazoyl-2)ethane hydrate was obtained having a melting point of 154°-155°C.

A 5-liter 3-necked flask equipped with a mechanical stirrer was charged with 2 liters of chloroform and 522 g (3 mole) of commercial grade 2,4-tolylenediisocyanate. To this stirred solution was added 270 g (1 mole) of stearyl alcohol over a period of 2 hours. After the addition, the contents of the flask were poured into 3 liters of hexane and cooled overnight. The resulting precipitate, N-(3-isocyanato-4-methylphenyl)octadecyl carbamate, was collected and reprecipitated from hexane and vacuum dried. The product had a melting point of 78°-79°C.

17.54 g (0.06 mole) of the previously formed 1,2-bis(5-amino-benzimidazoyl-2)ethane was placed into a 500 ml resin flask equipped with a mechanical stirrer together with 53.4 g (0.12 mole) of N-(3-isocyanato-4-methylphenyl)octadecyl carbamate in 573 g of HVI neutral oil having a viscosity of 70 at 210°F. This suspension was heated with stirring, under nitrogen, to 127°C. When the reaction was complete, the contents were cooled to approximately 110°C. The formulation was then milled three times in a three-roll paint mill. The resulting grease (Grease 1) contained 11.0% by weight thickener and had an ASTM unworked penetration ( $P_60$ ) of 212 and a worked penetration ( $P_{60}$ ) of 264.

#### EXAMPLE II

##### Preparation of Dibenzimidazole-Urea Thickening Agents

The procedure of Example I was essentially repeated except that 269 g (1 mole) of stearylamine was reacted with 2,4-tolylenediisocyanate in place of stearyl alcohol thereby forming N-(3-isocyanato-4-methylphenyl)octadecyl carbamide.

35.5 g (0.08 moles) of the carbamide intermediate was then reacted with 11.7 g (0.04 mole) of 1,2-bis(5-aminobenzimidazoyl-2)ethane prepared as in Example I in 382 g of a HVI neutral oil having a viscosity of 70 at 210°F. After completion of the reaction, the con-

15  
20  
25

15  
20  
25

30  
35

40

45

50

tents were cooled and milled three times in a three-roll paint mill. The resulting grease (Grease 2) contained 11.0% by weight thickener and had an ASTM unworked penetration ( $P_60$ ) of 268 and a worked penetration ( $P_{60}$ ) of 283.

#### EXAMPLE III

The procedure of Example I was essentially repeated except that a 60:40 molar ratio of stearyl and oleyl alcohols were employed in place of the stearyl alcohol reactant in Example I. The resulting grease contained 9.5% by weight thickener and had an ASTM unworked penetration ( $P_60$ ) of 197 and a worked penetration ( $P_{60}$ ) of 253.

#### EXAMPLE IV

The procedure of Example I was essentially repeated with the exception that an oligomerized alpha olefin synthetic hydrocarbon oil having a viscosity of 7.7 centistokes at 210°F was employed in place of the mineral lubricating oil. The resulting grease (Grease 4) contained 14% by weight thickener and had an ASTM unworked penetration ( $P_60$ ) of 242 and a worked penetration ( $P_{60}$ ) of 275.

#### EXAMPLE V

In order to demonstrate the excellent high temperature performance characteristics of the present grease compositions, the greases of Example I and III were subjected to two different high temperature bearing tests. The results of these tests are shown in the following table.

Table I

| Test Procedure                                                                                        | Grease 1 <sup>(1)</sup> | Grease 3 <sup>(1)</sup> |
|-------------------------------------------------------------------------------------------------------|-------------------------|-------------------------|
| Navy High Speed Bearing Test (Fed. Test Mtd. No. 331.1)<br>300°F, 10,000 rpm -<br>Bearing Life, Hours | 4322, 5118              | 4956+                   |
| ABEC Bearing Test (Fed. Test Mtd. No. 333) 350°F,<br>10,000 rpm -<br>Hours to Failure                 | 386 <sup>(2)</sup>      | 465 <sup>(2)</sup>      |

<sup>(1)</sup>Includes 1% wt phenyl-alpha-naphthylamine, 0.5% Oronite 250 (dilauryl selenide), 1% wt sodium sebacate and 0.03% wt 3-amino-1,2,4-triazole.

<sup>(2)</sup>Average of two runs.

#### EXAMPLE VI

Other dibenzimidazole thickeners and greases in accordance with the invention include those shown in the following table.

Table II

| Grease Com-<br>position | Acid or<br>Anhydride                                | Phenylene<br>Diamine               | Diisocyanate                                                | Alcohol<br>or Amine                                               | Base<br>Oil |
|-------------------------|-----------------------------------------------------|------------------------------------|-------------------------------------------------------------|-------------------------------------------------------------------|-------------|
| 5                       | Succinic<br>anhydride                               | 4-Nitro-o-<br>phenylene<br>diamine | 2,4-tolylene-<br>diisocyanate                               | 80% mole<br>$C_{18}H_{37}OH$                                      | A           |
| 6                       | Adipic<br>Acid                                      | 4-Nitro-o-<br>phenylene<br>diamine | 3,3-dimethyl-<br>diphenyl-<br>methane-4,4'-<br>diisocyanate | 20% mole<br>$C_{18}H_{37}NH_2$<br>100% mole<br>$C_{18}H_{37}NH_2$ | A           |
| 7                       | 1,2-Cyclo-<br>hexane di-<br>carboxylic<br>anhydride | 4-Nitro-o-<br>phenylene<br>diamine | 2,4-tolylene-<br>diisocyanate                               | 70% mole<br>$C_{20}H_{41}NH_2$                                    | B           |

Table II - Continued

| Grease<br>Com-<br>po-<br>sition | Acid or<br>Anhydride             | Phenylene<br>Diamine               | Diisocyanate                                    | Alcohol<br>or Amine                                                                                            | Base<br>Oil |
|---------------------------------|----------------------------------|------------------------------------|-------------------------------------------------|----------------------------------------------------------------------------------------------------------------|-------------|
| 8                               | Dodecyl<br>succinic<br>anhydride | 4-Nitro-o-<br>phenylene<br>diamine | 3,3-dimethyl-<br>biphenyl-4,4'-<br>diisocyanate | 30% mole<br>C <sub>12</sub> H <sub>25</sub> NH <sub>2</sub><br>100% mole<br>C <sub>18</sub> H <sub>37</sub> OH | B           |
| 9                               | Phthalic<br>anhydride            | 4-Nitro-o-<br>phenylene<br>diamine | 2,4-tolylene-<br>diisocyanate                   | 75% mole<br>C <sub>18</sub> H <sub>37</sub> OH<br>25% mole<br>C <sub>16</sub> H <sub>33</sub> OH               | C           |

Base Oil A - Mineral lubricating oil having a viscosity of 500 SSU at 100°F.

Base Oil B - Mineral lubricating oil having a viscosity at 70 SSU at 210°F.

Base Oil C - Mixture of hexadecyl isostearate and dimer acid esters.

I claim as my invention:

1. A dibenzimidazole compound corresponding to the formula:



wherein R<sub>1</sub> and R<sub>2</sub> are aliphatic hydrocarbyl radicals having six to 30 carbon atoms, R<sub>3</sub> is a hydrocarbylene radical having from two to 20 carbon atom, R<sub>4</sub> and R<sub>5</sub> are aromatic hydrocarbylene radicals having from six to 20 carbon atoms and X is —O— or



2. The compound of claim 1 wherein X is —O—.

3. The compound of claim 1 wherein X is

4. The compound of claim 1 wherein R<sub>3</sub> is an alkylene radical having two to 12 carbon atoms.5. The compound of claim 1 wherein R<sub>1</sub> and R<sub>2</sub> have from 12 to 24 carbon atoms.6. The compound of claim 5 wherein R<sub>4</sub> and R<sub>5</sub> are tolylene.7. The compound of claim 6 wherein R<sub>3</sub> is ethylene.8. The compound of claim 7 wherein R<sub>1</sub> and R<sub>2</sub> have 16 to 18 carbon atoms.

\* \* \* \* \*